

## UNITED STATES PATENT OFFICE.

VAHAN FENER, OF CHICAGO, ILLINOIS.

## ALLOY.

No Drawing.

Application filed January 14, 1926. Serial No. 81,314.

This invention relates to alloys and has for an object to produce an alloy of copper and tin in varying degrees of hardness, in its hardest state being adapted for tools or other devices ordinarily supposed to require tempered steel.

A further object of the invention is to provide a copper and tin alloy which can be produced in varying degrees of hardness for such purposes as bushings, bearings or electrical connections or work, the hardness of the metal to be controlled and determined by the requirements to which it is to be put and exhibiting as physical characteristics lowered elongation and reduction of area.

The hardness of the alloy is determined by the proportion of tin to the proportion of copper, the greater the amount of tin the harder the alloy.

As at present practiced the hardest alloy which seems desirable would be produced from 100 pounds of copper and 25 pounds of tin, whereas the softest alloy which seems feasible would be produced from 100 pounds of copper and 3 pounds of tin.

As a flux and for providing for the necessary tempering and uniting of the metals, ammonium chloride and potassium ferrocyanide are employed. The ingredients would be about as follows:

|                             | Hard.        | Soft.       |
|-----------------------------|--------------|-------------|
| Metallic copper.....        | 100 pounds.. | 100 pounds. |
| Metallic tin.....           | 25 pounds... | 3 pounds.   |
| Ammonium chloride.....      | 1 pound...   | 1 pound.    |
| Potassium ferrocyanide..... | 25 drachms   | 5 drachms.  |

The amount of ammonium chloride and potassium ferrocyanide above listed will be

varied and the exact amount employed will be determined by the action of the materials and is only approximate.

In carrying out the formation of this alloy, 100 pounds of copper is melted in any convenient or desired vessel. To the melted copper is added the tin, for the softest metal 3 pounds of the tin. Simultaneously with the adding of the tin, the ammonium chloride is added gradually, the metal being agitated during the addition of this ammonium chloride. The exact amount of ammonium chloride to be added is determined from the rising therefrom of a smoke or visible vapor and at the proper consistency the molten metal assumes a purplish color. After the metal assumes the purplish color, it is heated continuously for five minutes, agitation being continued all the time. After the expiration of five minutes, the molten mass is removed from heating and any film having arisen to the top of the molten metal is removed. The potassium ferrocyanide, about five drachms for the softest metal, is now added also during agitation which is continued thereafter for one or two minutes at which time the alloy is ready to pour into molds or any form desired.

What I claim to be new is:

An alloy comprising copper in the proportion of substantially 100 pounds to tin varying from 3 to 25 pounds, modified by the addition of ammonium chloride approximately one pound, and potassium ferrocyanide varying from 5 to 25 drachms while the metals are in molten condition.

In testimony whereof I affix my signature.

VAHAN FENER.